

## UNITED STATES PATENT OFFICE

2,541,692

## PAPER SIZE

August S. Ersperer, Spring Grove, Pa., assignor  
to P. H. Glatfelter Company, Spring Grove, Pa.,  
a corporation of Pennsylvania

No Drawing. Application January 14, 1947,  
Serial No. 722,071

10 Claims. (Cl. 260—26)

1

This invention relates to paper making and more particularly to a novel paper sizing composition and a method of making the size.

In the manufacture of papers that are resistant to ink and water penetration it has long been customary to incorporate in the paper stock that is to be used in making the paper a size that is adapted to inhibit the flow of ink and other liquids into the fibers of the paper. One widely used size comprises a relatively dilute alkaline dispersion or solution of rosin in water. The size is commonly incorporated into the paper stock in the beating operation prior to the forming of the paper into a sheet and a paper-makers' alum is added to cause the rosin to be precipitated upon the fibers of the paper stock.

The conventional rosin size is subject to a number of disadvantages. When such a conventional size is used the results are, at times, somewhat erratic, that is, the degree of resistance to ink penetration of the sized paper is non-uniform across or along the sheet. Also with certain types of paper there is a limit to the degree of sizing that can be obtained in that as the quantity of size is increased a point is reached at which further additions of size do not produce any increase in the resistance of the paper to ink penetration. Because of this limiting factor there are some cases in which it is not possible to obtain the desired sizing effect with a conventional rosin size. Moreover the large amounts of rosins present in hard-sized papers tend to lower the quality of the paper.

It is accordingly an object of the present invention to provide a paper size composition capable of overcoming the disadvantages of the conventional size. It is another object of the invention to provide a paper size that is capable of producing a relatively high degree of resistance to ink and water penetration. It is a further object of the invention to provide a paper size that can be used in substantially smaller amounts than the conventional rosin sizes and produce an equivalent sizing effect. It is still another object of the invention to provide a method of making such a size. Other objects and advantages of the invention will be in part obvious and in part pointed out hereafter.

The objects and advantages of the present invention may be achieved, in general, by incorporating in a paper size a quantity of a resin formed from a polyhydric alcohol and a polybasic acid, the character of the resin being such that it has a relatively high acid number. It has been found that penetration of ink through the paper and

2

spreading of ink along the surface of the paper may be inhibited by flocculating the coloring matter of the ink and that such flocculation of the coloring matter of the ink can be effectively produced by substances which have relatively high acid numbers, i. e., a relatively large number of acidic groups per unit molecular weight of the substance. Thus a suitable substance with a sufficiently high acid number when incorporated in a size under the proper conditions and applied to a sheet of paper will effectively increase the resistance of the paper to ink penetration.

It is evident that all substances having high acid numbers cannot be used since it is necessary that the substance used have not only a high acid number but that it also have chemical and physical properties which permit its effective incorporation in the paper without adversely affecting desirable properties of the paper other than resistance to ink penetration. It has been found that esters of polyhydric alcohols and polybasic acids, either in monomeric or polymeric form and having acid numbers of at least about 250 may be incorporated in a paper size which when applied to paper produces a material improvement in the resistance of the paper to ink penetration. It has been further found that a polymer of glycerol and maleic anhydride prepared under such conditions that its acid number is greater than about 350 is particularly effective in improving the ink penetration resistance of paper. The acid number of such a copolymer varies with the degree of polymerization of the copolymer be prepared in such manner that it is in a sufficiently low state of polymerization to give an acid number greater than 350.

The effectiveness of such a glycerol-maleic anhydride copolymer is such that it can be used in relatively small quantities and may, with advantage, be admixed with a relatively large proportion of rosin of paper making grade. The mixture of copolymer and rosin may then be dispersed in the usual manner and applied to the paper during the beating operation in the usual way.

In order to point out more fully the nature of the present invention the following specific example is given of a preferred method of compounding the size of the present invention. It is to be understood that the procedure set forth is illustrative only and may be modified in various ways as desired.

A mixture is prepared of 305 pounds of rosin of paper making grade and 25 pounds of a copolymer of glycerol and maleic anhydride having an

acid number in excess of 350. The temperature of the mixture is raised to 140° to 150° C. to ensure complete melting of the ingredients and the resin mixture is then mixed vigorously by mechanical agitation. The resulting mixture is neutralized with an alkaline solution made up by dissolving 60 pounds of soda ash in 20 gallons of water. The alkaline solution is added to the mixture slowly with continuous agitation and with the simultaneous addition of water that has been heated to a temperature of 70° to 80° C. The hot water is added to prevent the mixture from getting too thick and the quantity added is that amount which is sufficient to keep the mixture in a conveniently fluid condition.

When all of the alkali has been added the mixture is further diluted with hot water at 70° to 80° C. to a total volume of approximately 100 gallons and it is then further diluted with either warm or cold water to a total volume of 330 gallons.

The resulting size dispersion or solution contains about 12% by weight of solids or roughly one pound per gallon, and its pH is approximately 9. The size as thus prepared is in condition to be added to the beater in the usual way.

It may be pointed out that useful products are obtained in various intermediate stages of the foregoing procedure. Thus the mixture of rosin and copolymer may be cooled until it solidifies and stored as such for later use or it may be shipped to a point at which it is to be used and subsequently neutralized and dispersed in water. Also the size may be stored or shipped in relatively concentrated form and diluted to its final concentration at the time that it is to be used.

The quantity of the copolymer admixed with the rosin may be varied through a relatively wide range. I have found that desirable results are obtained by incorporating from about 5% to about 25% by weight of copolymer in the rosin-copolymer mixture. Within this range of proportions the composition that I prefer to use comprises about 10% by weight of the copolymer and 90% by weight of the rosin.

It has been found that a size prepared as described above is substantially more effective than conventional rosin sizes in inhibiting penetration of ink into papers that have been sized therewith. A variety of papers sized with the size of the present invention have been tested by a standard ink penetration test and it has been found that the precise degree of improvement varies somewhat with the type of paper to which the size is applied. However an appreciable increase in ink penetration resistance was found in the case of all papers tested and in some cases the ink resistance was more than double that obtained with a conventional rosin size when corresponding quantities of the two sizes were used. Thus it is possible to use substantially smaller quantities of the present size and still obtain a sizing effect equivalent to that obtained with a conventional rosin size.

Since many embodiments might be made of the present invention and since many changes might be made in the embodiment disclosed herein, it is to be understood that the foregoing description is to be interpreted as illustrative only and not in a limiting sense.

I claim:

1. A paper size composition comprising an aqueous alkaline dispersion of a mixture of rosin and an ester of glycerol and maleic anhydride, said ester having an acid number of at least 250.

2. A paper size composition comprising an aqueous alkaline dispersion of a mixture of rosin and a copolymer of glycerol and maleic anhydride, the degree of polymerization of said copolymer being sufficiently low that the acid number of said copolymer is greater than 350.

3. A paper size composition comprising an aqueous alkaline dispersion of a mixture of rosin and a copolymer of glycerol and maleic anhydride, said copolymer being present to the extent of between 5% and 25% by weight of said mixture and the degree of polymerization of said copolymer being sufficiently low that the acid number of said copolymer is greater than 350.

4. A paper size composition comprising an aqueous alkaline dispersion of a mixture of rosin and a copolymer of glycerol and maleic anhydride, said copolymer being present to the extent of about 10% by weight of said mixture and the degree of polymerization of said copolymer being sufficiently low that the acid number of said copolymer is greater than 350.

5. A paper size composition comprising an aqueous alkaline dispersion containing about 12% by weight of a mixture of rosin and a copolymer of glycerol and maleic anhydride, the degree of polymerization of said copolymer being sufficiently low that the acid number of said copolymer is greater than 350.

6. A paper size composition comprising a mixture of rosin and a copolymer of glycerol and maleic anhydride, the degree of polymerization of said copolymer being sufficiently low that the acid number of said copolymer is greater than 350.

7. A paper size composition comprising a mixture of rosin and a copolymer of glycerol and maleic anhydride, said copolymer being present to the extent of between 5% and 25% by weight of said mixture and the degree of polymerization of said copolymer being sufficiently low that the acid number of said copolymer is greater than 350.

8. A paper size composition comprising a mixture of rosin and a copolymer of glycerol and maleic anhydride, said copolymer being present to the extent of about 8% by weight of said mixture and the degree of polymerization of said copolymer being sufficiently low that the acid number of said copolymer is greater than 350.

9. The method of making a paper size which comprises mixing together in the molten state rosin and a copolymer of glycerol and maleic anhydride in a sufficiently low state of polymerization that its acid number is greater than 350 and adding to said molten mixture an aqueous solution of an alkali to disperse said mixture.

10. A paper size composition comprising an aqueous alkaline dispersion of a copolymer of glycerol and maleic anhydride, the degree of polymerization of said copolymer being sufficiently low that the acid number of said copolymer is greater than 350.

AUGUST S. ERSPAMER.

#### REFERENCES CITED

The following references are of record in the file of this patent:

#### UNITED STATES PATENTS

| Number    | Name     | Date          |
|-----------|----------|---------------|
| 1,413,144 | Weisberg | Apr. 18, 1922 |
| 1,780,375 | Bradley  | Nov. 4, 1930  |

**Certificate of Correction**

Patent No. 2,541,692

February 13, 1951

**AUGUST S. ERSPAMER**

It is hereby certified that error appears in the printed specification of the above numbered patent requiring correction as follows:

Column 2, line 34, after the word "copolymer" insert *and becomes smaller as the degree of polymerization increases. Hence it is desirable that the co-polymer;*

and that the said Letters Patent should be read as corrected above, so that the same may conform to the record of the case in the Patent Office.

Signed and sealed this 5th day of June, A. D. 1951.

[**SEAL**]

**THOMAS F. MURPHY,**  
*Assistant Commissioner of Patents.*